

1

2,940,852

## m,m'-DIOXYDIPHENOLS AS COUPLING COMPONENTS IN DIAZOTYPE INTERMEDIATES OF HIGH OPACITY

Clifford E. Herrick, Jr., Chenango Forks, and Chester E. Slimowicz, Vestal, N.Y., assignors to General Aniline & Film Corporation, New York, N.Y., a corporation of Delaware

No Drawing. Filed Feb. 19, 1957, Ser. No. 641,023

7 Claims. (Cl. 96—91)

The present invention relates to light sensitive diazotype materials containing m,m'-dioxydiphenols as coupling components and, particularly to diazotype intermediates of high opacity containing such coupling components.

One of the most widely used techniques in the diazotype reproduction art involves the use of the so-called intermediate or transition print. Thus, in place of making a large number of copies from a frail or valuable original, it is customary to make a single copy on an intermediate diazotype paper or foil. This intermediate diazotype is then used as the photo master for the production of additional prints.

There are many advantages in the use of an intermediate master. Wear and tear on a frail original are avoided. Owing to the high contrast of the diazotype process, some improvement in image density can usually be realized in the intermediate print, especially if the original itself be dirty or old. Furthermore, the speed at which copies can be made is substantially greater than when the original itself is used as a photo master, a fact attributable to the higher transparency of the foil base compared to the original base.

A variety of useful techniques using intermediate foil masters have been evolved, such as overlay printing, partial eradication of the original image, etc. Consequently, the production of a satisfactory intermediate material is a very basic and important part of diazotype technology.

In order to be satisfactory as an intermediate material, a diazotype layer must meet rigid and diverse specifications. The intermediate foil should have the fastest possible printing speed consistent with good opacity, and form a dye having both good actinic opacity and good visual opacity, since visual examination of the intermediate is frequently necessary. The layer must exhibit satisfactory stability, both in the package and in the developed foil. Both the packaged and developed foil must show good stability against yellowing, especially yellowing which occurs on exposure of a developed foil to ultra-violet radiation since such yellowing increases the opacity of the material. The dye formed should be free from a tendency to migrate or to offset when in contact with other materials. Heretofore, it has not been possible to combine all of these properties to a satisfactory degree in any commercial product.

One of the most widely used azo dye coupling components in diazo intermediate products is resorcinol. When freshly coated in high concentration, resorcinol yields a dye having good actinic opacity. However, as the coated material ages, diffusion and redistribution of the components takes place so that in place of the mono-azo coupling originally predominant, bis-coupling becomes important. Resorcinol is thus very sensitive to the diazo/coupler ratio. Consequently, as the material ages, the visual opacity increases as the result of bis-dye formation while a marked falling off in actinic opacity occurs at the same time. In addition, with the diazos most suit-

2

able for the production of high actinic opacity, resorcinol is too active a coupler especially at the higher coupler concentration which leads predominantly to mono-azo coupling and such layers cannot be satisfactorily stabilized against precoupling.

On the other hand, coupling components are known which provide layers of good stability having good actinic opacity of which m-hydroxyphenylurea and dimethylaminomethyl-2,5-xylenol are examples. These materials, however, suffer from restricted solubility, are prone to offset under certain circumstances, and yield layers which fail to develop the dye images rapidly and completely on exposure to ammonia. In addition, their visual opacity is poor.

15 Among the host of materials studied as coupling components for diazotype intermediates, the 2,6-dialkoxy- and-dialkyl phenols as well as the resorcinol monoethers disclosed in U.S. Patent 2,516,931 have been found excellent in many respects in that they yield layers having 20 good stability towards precoupling, have good actinic opacity and better than average visual opacity. These materials, however, are often liquids or semi-solids and frequently have an offensive and penetrating medicinal odor. These properties have precluded their use in commercial materials.

We have now found that certain polyfunctional derivatives of the resorcinol monoether class, i.e., m,m'-dioxydiphenols, are especially well adapted for use as couplers in intermediate materials. These couplers possess an 30 unusual combination of satisfactory visual and high actinic opacity and freedom from objectionable odor. A further advantage of the high actinic opacity afforded by this class of derivatives is that it permits the use of shading couplers for the purpose of enhancing even further the 35 visual opacity without seriously compromising the actinic opacity requirements. Such a course is not practical with couplers which yield intermediate prints possessing mediocre or at best only acceptable actinic opacity. The new materials have excellent solubility in solvents. They form 40 layers free from color shift on aging and yield dyes which are less prone to migrate than the dyes formed by the simple monoethers. An especially surprising discovery is the fact that while these polyfunctional derivatives are 45 readily stabilized against precoupling, they ammonia-develop readily and completely. In fact, their precoupling activity is so low that it is possible to combine them satisfactorily with a class of diazo compounds, namely, the p-4-morpholinylbenzenediazocomplexes which heretofore were unusable owing to their great coupling activity, to produce foils of outstandingly high printing speed and whose dye images possess outstanding actinic opacity. The result is a foil which sets a new standard owing to its 50 high printing speed and actinic opacity and above average visual density in the diazotype art.

55 Light sensitive diazotype materials containing m,m'-dioxydiphenols as coupling components and, more particularly, those intermediate materials of high opacity containing such couplers constitute the purposes and objects of the present invention.

60 The polyfunctional resorcinol ethers contemplated herein may be depicted by the following general formula:



in which A is alkylene such as ethylene, trimethylene, tetramethylene, pentamethylene, methyltrimethylene; alkylenearylenealkylene, i.e., methylenephenylenemethylene, ethylenephenyleneethylene and the like; isoalkylidene such as isopropylidene and the like; X and Y are hydrogen, alkyl such as methyl, ethyl, butyl, amyl, hexyl and the like; sulfo, halogen such as chlorine and bromine; p is 0 or a whole number; and n is 1 when p is 0 and p + 1 when p is a whole number, i.e., 2 when p is 1.

The following examples will serve to illustrate the invention but it is to be understood that the invention is not restricted thereto.

*Example I*

|                                                                       |      |     |    |
|-----------------------------------------------------------------------|------|-----|----|
| Methanol                                                              | mls. | 57  | 15 |
| Acetone                                                               | mls. | 40  |    |
| Methyl "Cellosolve" acetate                                           | mls. | 3   |    |
| Sulfosalicylic acid                                                   | gms. | 1   |    |
| Thiourea                                                              | gms. | .4  | 20 |
| Zinc chloride                                                         | gms. | .6  |    |
| m,m'-Ethylenedioxydiphenol                                            | gms. | 1.5 |    |
| 4-ethylamino-3-methylbenzenediazonium chloride: zinc chloride complex | gms. | 1.9 |    |

When this solution was coated on a starch-filled cloth base which had been surface-coated with a polyvinyl acetate or on plastic-coated cloth or cellulose acetate foil base, dried, exposed to actinic light under a positive original, and treated with ammonia vapors, a yellowish-brown positive copy was obtained having good visual density and excellent actinic opacity.

The m,m'-ethylenedioxydiphenol was made by a modification of the method of Kohn and Wilhelm (Monatshefte, 43, 545-55 (1923)), from resorcinol, ethylene bromide, and aqueous sodium hydroxide.

*Example II*

|                                                                 |      |     |    |
|-----------------------------------------------------------------|------|-----|----|
| Water                                                           | mls. | 45  | 40 |
| Isopropyl alcohol                                               | mls. | 40  |    |
| Formic acid                                                     | mls. | 15  |    |
| Citric acid                                                     | gms. | 3.5 |    |
| Sulfosalicylic acid                                             | gms. | 2   |    |
| Aluminum sulfate                                                | gms. | 3.5 | 45 |
| m,m'-Ethylenedioxydiphenol                                      | gms. | 2.5 |    |
| p-4-morpholinylbenzenediazonium chloride: zinc chloride complex | gms. | 7   |    |

When this composition was coated on precoated glass cloth base, dried, irradiated with actinic light under a positive original, and exposed to ammonia vapors, it gave a yellowish-brown positive copy with excellent opacity to ultraviolet light, fade resistance, and stability.

*Example III*

|                                                  |      |     |    |
|--------------------------------------------------|------|-----|----|
| Water                                            | mls. | 56  |    |
| Isopropyl alcohol                                | mls. | 22  |    |
| Gamma-butyrolactone                              | mls. | 4   | 60 |
| Butanol                                          | mls. | 4   |    |
| Citric acid                                      | mls. | 2   |    |
| Formic acid                                      | mls. | 5   |    |
| Phosphoric acid                                  | mls. | 1.3 |    |
| Thiourea                                         | gms. | 3.5 | 65 |
| Zinc chloride                                    | gms. | 0.6 |    |
| m,m'-Ethylenedioxydiphenol                       | gms. | 6.5 |    |
| p-4-ethylamino-3-methylbenzenediazonium fluoride | gms. | 12  |    |

When coated on cellulose acetate foil base, dried, exposed to actinic light under a positive original, and treated with ammonia vapors, this composition yielded a yellowish-brown image with good visual density, opacity to ultraviolet light, dye stability, and developability.

*Examples IV*

|                                                                 |      |     |
|-----------------------------------------------------------------|------|-----|
| Methyl "Cellosolve"                                             | mls. | 60  |
| Methyl "Cellosolve" acetate                                     | mls. | 10  |
| Sulfosalicylic acid                                             | gms. | 2   |
| Phosphoric acid                                                 | mls. | .3  |
| Citric acid                                                     | gms. | .5  |
| Formic acid                                                     | mls. | 20  |
| m,m'-Ethylenedioxydiphenol                                      | gms. | 3.2 |
| p-4-morpholinylbenzenediazonium chloride: zinc chloride complex | gms. | 2.5 |

When coated on cellulose acetate foil base, dried, irradiated with actinic light under a positive original, and exposed to ammonia vapors, this composition yielded a yellowish-brown image with excellent stability and good visual density. The printing speed and ultraviolet opacity of this material were outstanding.

*Example V*

The procedure is the same as in Example I excepting that the coupling component used is m,m'-trimethylenedioxydiphenol of the following formula:



This compound may be prepared by the method of Kohn and Wilhelm (Monatshefte 43, 545-5 (1923)). A more convenient laboratory method, however, is the reaction of m-nitrophenol with trimethylene bromide and alkali to give 3,3'-dinitrotetramethylenedioxydiphenene, M. 121-3° C., which was reduced catalytically in ethanol over palladium on carbon to yield m,m'-ethylenedioxydiphenol, M. 151-3° C. Diazotization and hydrolysis with dilute sulfuric acid gave a product identical with the compound prepared by Kohn and Wilhelm (I.c.).

*Example VI*

The procedure is the same as in Example II excepting that the coupling component used is m,m'-tetramethylenedioxydiphenol of the following formula:



This compound may be prepared as follows: m-Nitrophenol was reacted with 1,4-dibromobutane to give 3,3'-dinitrotetramethylenedioxydiphenene, M. 135-7° C., which was reduced in isopropyl alcohol over palladium on carbon to the amine, M. 128-30° C. Diazotization and hydrolysis with dilute sulfuric acid were completed as in Example V and the desired compound was obtained as colorless needles, M. 105-8° C.

*Example VII*

The procedure is the same as in Example III excepting that the coupling component is m,m'-pentamethylenedioxydiphenol of the following formula:



This compound may be prepared as follows: 1,5-dibromopentane and m-nitrophenol were condensed to 3,3'-dinitropentamethylenedioxydiphenene, M. 94-6° C. This was reduced in ethyl alcohol over palladium on carbon to the amine, M. 119-21° C. Diazotization and hydrolysis with dilute sulfuric acid gave the desired compound as colorless needles, M. 110-1° C. After recrystalliza-

tion from benzene, the product melted at 110.5-12° C., and analyzed as follows: C 70.98, H 6.94; calculated C 70.86, H 6.94.

*Example VIII*

The procedure is the same as in Example I excepting that the coupling component employed is *m,m'*-1-methyltrimethylenedioxydiphenol of the following formula:



This compound may be prepared as follows: *m*-Nitrophenol and 1,3-dibromobutane are reacted in the presence of alkali to give 3,3'-dinitro-1-methyltrimethylenedioxydiphenol, M. 73-7° C. This was reduced in ethanol over palladium on carbon and was isolated as the amine hydrochloride, M. 228-31° C., by passing anhydrous hydrogen chloride through the ethanol solution of the free amine. Diazotization and hydrolysis with dilute sulfuric acid gave a viscous oil which was distilled, B<sub>13</sub> 95-135° C., but which resisted crystallization.

*Example IX*

The procedure is the same as in Example III excepting that the coupling component is 6,6'-dimethyl-3,3'-trimethylenedioxydiphenol of the formula:



This compound may be prepared as follows: 3-nitro-4-methylphenol was prepared from 3-nitro-4-methylaniline by diazotization and hydrolysis (Harvey and Robertson, J. Chem. Soc. 1938, 97-101). This was reacted with trimethylene bromide and alkali to yield 4,4'-dimethyl-3,3'-dinitrotrimethylenedioxydiphenol, M. 106-9° C. Reduction in ethanol over palladium on carbon went smoothly to give the amino derivative, M. 129-30° C. Diazotization and hydrolysis by the usual method gave the desired compound, M. 139-41° C.

*Example X*

The procedure is the same as in Example III excepting that the coupling component is *m,m'*-(*p*-phenylene-dimethylenedioxy)diphenol of the formula:



This compound may be prepared as follows: *m*-Nitrophenol and *p*-phenylenedimethylene bromide were reacted to give 3,3'-dinitro-*p*-phenylenedimethylenedioxydiphenol, M. 193-6° C. The amino compound, prepared by reduction in ethanol over palladium on carbon was diazotized and hydrolyzed to the desired compound, M. 72-4° C.

*Example XI*

The procedure is the same as in Example II excepting that the coupling component is 6,6'-dihexyl-3,3'-isopropylidenedioxydiphenol of the formula:



This was prepared from 4-hexylresorcinol, acetone, and hydrogen chloride by the method of Uoto and Makida (Jap. Pat. 289 (Jan. 30, 1951); Chem. Abstr., 47, 4369g (1953)).

The procedure is the same as in Example I excepting that the coupling component employed is *m,m'*-ethylene-dioxydiphenol-formaldehyde polymer of the formula:



This was formed in an attempted Mannich reaction between *m,m'*-ethylenedioxydiphenol, formalin, and diethylamine in ethanol. The product was a semi-solid which was soluble in alkali, insoluble in acid, was free of combined nitrogen, and depressed the melting point of *m,m'*-ethylenedioxydiphenol. In this formula *p* is a whole number and *n* is *p*+1.

*Example XII*

The procedure is the same as in Example II excepting that the coupling component employed is 4,4',6,6'-tetramethyl-3,3'-trimethylenedioxydiphenol of the formula:



This compound may be prepared as follows: 2,4-dimethyl-5-nitrophenol was obtained as indicated by Robertson and Robinson, J. Chem. Soc., 2201 (1927), and reacted with trimethylenebromide and alkali to give 5,5'-dinitro-2,2',4,4'-tetramethyltrimethylenedioxydiphenol, M. 171-4° C. This reduced smoothly over palladium on carbon to the diamine, M. 112-15° C. Diazotization and hydrolysis with dilute sulfuric acid gave the desired compound, M. 142.5-4.5° C.

Modifications of the invention will occur to persons skilled in the art and we, therefore, do not intend to be limited in the patent granted except as necessitated by the appended claims.

We claim:

1. Light sensitive diazotype materials comprising a base sensitized with a light sensitive diazonium compound, and as the coupling component, the compound of the following formula:



wherein A is selected from the class consisting of alkylene, alkylene-arylene-alkylene and isalkylidene; X and Y are selected from the class consisting of hydrogen, alkyl, sulfo and halogen; p is selected from the class consisting of 0 and a whole number; and n is 1 when p is 0 and p+1 when p is a whole number.

2. Light sensitive intermediate diazotype materials comprising a translucent base sensitized with a light sensi-

tive diazonium compound, and as the coupling component, a compound of the following formula:



10

wherein A is selected from the class consisting of alkylene, alkylene-arylene-alkylene and isoalkylidene; X and Y are selected from the class consisting of hydrogen, alkyl, sulfo and halogen; p is selected from the class consisting of 0 and a whole number; and n is 1 when p is 0 and p+1 when p is a whole number.

3. The article as defined in claim 2 wherein the coupling component is m,m'-ethylenedioxydiphenol.

4. The article as defined in claim 2 wherein the coupling component is m,m'-ethylenedioxydiphenol and the

15

5

6

7

8

light sensitive compound is a p-4-morpholinylbenzene diazonium salt.

5. The article as defined in claim 2 wherein the coupling component is m,m'-trimethylenedioxydiphenol.

6. The article as defined in claim 2 wherein the coupling component is m,m'-tetramethylenedioxydiphenol.

7. The article as defined in claim 2 wherein the coupling component is m,m'-pentamethylenedioxydiphenol.

#### References Cited in the file of this patent

##### UNITED STATES PATENTS

|           |                  |               |
|-----------|------------------|---------------|
| 2,536,989 | Von Glahn et al. | Jan. 2, 1951  |
| 2,650,925 | Urne             | Sept. 1, 1953 |

##### FOREIGN PATENTS

|         |               |               |
|---------|---------------|---------------|
| 626,391 | Great Britain | July 14, 1949 |
|---------|---------------|---------------|

##### OTHER REFERENCES

Chem. Abstracts, 47, 4369g (1953).

Monatshefte, 43, 545 to 55 (1923).

Saunders, The Aromatic Diazo, 2nd ed., 1949, pub. by Edward Arnold & Co., London, pages 197-200 and 217-219.